# EUROPEAN PATENT SPECIFICATION

(11) **EP 0 608 406 B1**
(45) Date of publication and mention of the grant of the patent: **22.01.1997**
(21) Application number: 93917987.5
(22) Date of filing: 04.08.1993
(51) Int. Cl.: A43B 23/07, A43B 17/10

(54) **SHOE LINING FABRICS**
SCHUHINNENGEWEBE
ETOFFES POUR DOUBLURE DE CHAUSSURE

(30) Priority: 05.08.1992 GB 9216632
(43) Date of publication of application: 03.08.1994
(73) Proprietor: E.I. DU PONT DE NEMOURS & COMPANY INCORPORATED, Wilmington Delaware 19898 (US)
(72) Inventor: TRAVIS, Anthony 2 Newlands Road, Cumbria CA13 0AH (GB); BOARDMAN, Graham 1 Spring Bank Meadow, North Yorkshire HG4 1HQ (GB)
(74) Representative: Abitz, Walter, Dr.-Ing.
(86) International application number: GB9301647
(87) International publication number: WO9403081

(56) References cited:
- EP-A- 0 432 282
- DE-A- 2 447 178
- DE-A- 3 520 093
- US-A- 4 607 439

## Description

This invention relates to a fabric, in particular a fabric which has improved characteristics in terms of moisture transfer.

DE-A-35 20 093 relates to an insole comprising an absorbent layer of moisture-storing fibers as well as a moisture-permeable layer of textile material affixed thereto.

DE-A-24 47 178 relates to a shoe inner sole, especially an insole, having an air-permeable base structure.

One of the main problems connected with a fabric which is worn under conditions where a high degree of moisture in the form of perspiration is likely to be produced is that unless perspiration is removed from the surface of the body, the wearer can suffer considerable discomfort.

It is known that this problem can be solved by a fabric knitted from polyamide 66 yarn and cotton such that the polyamide forms one surface and the cotton the other. In use, the polyamide lies adjacent the moisture source, the moisture being wicked away from the source and into the cotton from which it evaporates.

This solution is satisfactory where evaporation can take place freely. However, there is still a problem when the fabric is not in contact with atmosphere, for example where the fabric is used as an inner lining in footwear where even if the outer layer can breath, ie has a degree of porosity to vapour, rapid evaporation is not possible and discomfort ray be caused if moisture is produced faster than it can evaporate.

It is an object of this invention to provide a fabric which allows removal of moisture from the surface which is adjacent the moisture source and which is capable of "storing" the moisture remote from said surface whilst the fabric is in "use" ie whilst a shoe is being worn and which will, when the fabric is not in "use" ie when the shoe is removed, allow evaporation of the moisture through the surface normally adjacent the moisture source so that the fabric can dry rapidly.

According to one aspect of the invention, there is provided a fabric comprising the features of claim 1.

The layers may be laminated together by any suitable means that will allow passage of moisture. A preferred method is to spray a moisture-cured polyurethane adhesive from a highly volatile solvent such as methylene chloride, the rapid evaporation of the solvent giving a high degree of porosity to the adhesive layer.

According to a preferred aspect of the invention, the second layer is formed from heat bonded, polyamide 66/6, core-sheath heterofilaments.

The lower the decitex per filament (dpf) of the yarn, the more efficient is the wicking action. However, the abrasion resistance of the fabric is also lowered and may not be sufficient for use in shoe linings.

According to a further aspect of the invention, the first layer is formed from two yarns having differing dpf's, such that the higher dpf yarn lies in the surface adjacent the moisture source and the lower dpf yarn lies in the surface remote from the moisture source.

However, perfect separation of the yarns in this way can only be achieved easily using a double jersey knitting machine.

Surprisingly it has been found that effective wicking takes place even if the surface is formed from both yarns.

Hence according to a further aspect of the invention the higher dpf yarn need only form a major part of the surface of the layer.

Preferably the yarns have dpf's in the range 3 to 5, specifically 4, and 1 to 2, specifically 1.7, respectively.

The invention will be more readily understood from the following examples.

### Example 1

A fabric was knitted on a single jersey knitting machine from false twist textured, 78f46, trilobal polyamide 66 yarn, ie yarn consisting of 46 filaments each having a decitex of 1.7, the filaments having a trilobal cross-section.

One surface of the fabric was sprayed with moisture curing polyurethane adhesive dissolved in methylene chloride and then bonded to a non-woven fabric formed from nylon 66/6 core/sheath heterofil and having an area weight of 120g/sq.m.

A drop of water having a diameter of approximately 5mm and containing a small amount of dye was placed on the knitted surface of the combined fabrics. It was immediately absorbed with virtually no sideways spreading and a comparison of the knitted and non-woven surfaces showed that the knitted surface was the drier.

In comparison, when a similar drop was placed on the surface of the knitted fabric alone and the non-woven fabric alone, the water spread rapidly sideways and in each case the surface was damper than the knitted surface of the combined fabrics.

### Example 2

Example 1 was repeated except that the knitted fabric was produced on a double jersey machine from false twist textured, 78f20, circular, polyamide yarn and the 78f46 yarn of Example 1, with the 78f46 yarn forming the surface bonded to the non-woven fabric.

Similar results were obtained and indeed there was little difference, in terms of the spreading and relative dampness of the surfaces, between the combined fabrics and the knitted fabric alone.

Samples, having a diameter of 2cm, of the knitted fabric alone and the combined fabrics were weighed. Water was then dripped evenly over the surface of the samples until saturation was reached. The samples were weighed again and it was found that the combined fabrics had absorbed more than 3 times as much water as the knitted fabric alone.

### Example 3

Example 2 was repeated except that the knitted fabric was produced on a single jersey machine such that the 78f20 yarn formed a major portion of the non-bonded surface.

Similar results were obtained except that a slightly greater spreading of the drop was evident.

### Example 4

The combined fabrics of Examples 1,2 and 3 were tested for abrasion resistance using a standard Martindale Tester. The results showed that the fabric of Example 1 had considerably less resistance than the fabrics of Examples 2 and 3 which showed similar resistance.

### Example 5

Four conventional training shoes(A,B,C and D), lined respectively with the combined fabrics of Examples 1,2 and 3, and the non-woven fabric alone, were weighed, filled with water to saturate the linings, emptied and weighed again and then stored at 20°C. Further weighings were carried out after 3, 7 and 12 hours. The results are shown in the Table.

**TABLE**

| SHOE | % WATER REMAINING | | | |
|---|---|---|---|---|
| | 0 HOURS | 3 HOURS | 7 HOURS | 12 HOURS |
| A | 100 | 56 | 39 | 0 |
| B | 100 | 57 | 38 | 0 |
| C | 100 | 57 | 36 | 0 |
| D | 100 | 42 | 10 | 0 |

## Claims

1. A fabric comprising a first knitted or woven layer laminated to a second non-woven layer, characterized in that said first layer is formed from two yarns of differing decitex per filament, such that the yarn having the higher decitex per filament forms the major portion of the surface remote from the second layer, whereby moisture is drawn away from the surface adjacent a moisture source through the first layer into the second layer which acts as a reservoir for the moisture.

2. A fabric according to claim 1, in which the layers are laminated together by a moisture-cured polyurethane spray applied from a volatile solvent.

3. A fabric according to claim 1 or 2, in which the second layer is formed from heat bonded, polyamide 66/6, core-sheath heterofilaments.

4. A fabric according to claim 1, 2, or 3, in which the lower decitex per filament yarn is formed from polyamide 66 yarn having a decitex per filament of 1.7.

5. A fabric according to claim 1, in which the higher decitex per filament yarn forms all of the surface remote from the second layer and the lower decitex per filament yarn forms all of a surface adjacent the second layer.

6. A fabric according to claim 1, in which one yarn has a decitex per filament in the range 3 to 5 and the other yarn has a decitex per filament of 1 to 2.

7. A fabric according to claim 6, in which one yarn has a decitex per filament of 4 and the other yarn has a decitex per filament of 1.7.

## Patentansprüche

1. Textilstoff, umfassend eine erste Gestrick- oder Gewebeschicht, die auf eine zweite Schicht aus Faservliesstoff aufkaschiert ist, dadurch gekennzeichnet, daß die erste Schicht aus zwei Garnen mit unterschiedlichen dtex-Werten pro Filament gebildet wird, so daß das Garn mit dem höheren dtex-Wert pro Filament den größeren Teil der von der zweiten Schicht entfernten Fläche bildet, wodurch Feuchtigkeit aus der an einer Feuchtigkeitsquelle anliegenden Fläche durch die erste Schicht hindurch in die zweite Schicht abgezogen wird, die als Speicher für die Feuchtigkeit wirkt.

2. Textilstoff nach Anspruch 1, bei dem die Schichten zusammenkaschiert werden durch ein wassergehärtetes Spray aus Polyurethan, das aus einem flüchtigen Lösungsmittel aufgebracht wird.

3. Textilstoff nach Anspruch 1 oder 2, bei dem die zweite Schicht aus wärmegebundenen Kern-Mantel-Heterofilamenten aus Polyamid 66/6 gebildet wird.

4. Textilstoff nach Anspruch 1, 2 oder 3, bei dem sich das Garn mit dem niedrigeren dtex-Wert pro Filament aus Garn aus Polyamid 66 mit einem dtex-Wert von 1,7 pro Filament besteht.

5. Textilstoff nach Anspruch 1, bei dem das Garn mit dem höheren dtex-Wert pro Filament die gesamte von der zweiten Schicht entfernte Fläche bildet und das Garn mit dem niedrigeren dtex-Wert pro Filament die gesamte an der zweiten Schicht anliegende Fläche bildet.

6. Textilstoff nach Anspruch 1, bei dem ein Garn einen dtex-Wert im Bereich von 3 bis 5 pro Filament aufweist und das andere Garn einen dtex-Wert von 1 bis 2 pro Filament aufweist.

7. Textilstoff nach Anspruch 6, bei dem ein Garn einen dtex-Wert von 4 pro Filament aufweist und das andere Garn einen dtex-Wert von 1,7 pro Filament aufweist.

## Revendications

1. Un tissu comprenant une première couche tissée ou tricottée stratifiée sur une seconde couche non-tissée caractérisé en ce que ladite première couche est formée de deux fils de décitex par filament différent, de façon telle que le fil ayant le décitex par filament le plus élevé constitue la majeure partie de la surface à l'opposé de la seconde couche, grâce à quoi l'humidité est éliminée de la surface en contact avec une source d'humidité à travers la première couche dans la seconde couche qui sert de réservoir pour l'humidité.

2. Un tissu selon la revendication 1 dans lequel les couches sont stratifiées ensemble à l'aide d'une pulvérisation de polyuréthane durcissant à l'humidité appliquée avec un solvant volatil.

3. Un tissu selon la revendication 1 ou 2, dans lequel la seconde couche est formée d'hétérofilaments de polyamide 66/6, liés thermiquement, de type âme/enveloppe.

4. Un tissu selon la revendication 1, 2 ou 3, dans lequel le fil de décitex par filament le plus faible est constitué de fil de polyamide 66 ayant un décitex par filament de 1,7.

5. Un tissu selon la revendication 1, dans lequel le fil de décitex par filament le plus élevé forme la totalité de la surface opposée à la seconde couche et le fil de décitex par filament le plus faible forme la totalité d'une surface en contact avec la seconde couche.

6. Un tissu selon la revendication 1, dans lequel un fil présente un décitex par filament de 3 à 5, et l'autre fil a un décitex par filament de 1 à 2.

7. Un tissu selon la revendication 6, dans lequel un fil a un décitex par filament de 4 et l'autre fil a un décitex par filament de 1,7.
